

## UNITED STATES PATENT OFFICE

2,303,405

## ALLOY

Cecil Spencer Sivil, Roselle, N. J., assignor to  
Baker & Company, Inc., Newark, N. J., a corpora-  
tion of New Jersey

No Drawing. Original application December 20,  
1941, Serial No. 423,793. Divided and this ap-  
plication June 9, 1942, Serial No. 446,383

3 Claims. (Cl. 75—172)

This invention relates to alloys and is con-  
cerned in particular with platinum metal alloys.

It is one object of my invention to provide  
alloys of great corrosion resistance, high melt-  
ing point and great hardness and strength. It  
is another object of my invention to provide such  
alloys of great electrical resistance. It is a fur-  
ther object of my invention to provide such alloys  
of low specific gravity and low cost.

This application is a division of my applica-  
tion Serial No. 423,793, filed December 20, 1941,  
which in turn is a continuation in part of my  
application Serial No. 401,653, filed July 9, 1941,  
which in turn is a continuation in part of my ap-  
plication Serial No. 378,376, filed February 11, 15

In my aforesaid, co-pending application No.  
423,793 I have described alloys of 60% to about  
95% palladium, 0.5% to 20% ruthenium, and  
2.5% to 39.5% iridium. The alloys according  
to this invention comprise palladium, ruthenium,  
iridium, and rhodium. In such alloys the pal-  
ladium content may be as low as about 60% and  
as high as about 94.5%, the ruthenium content  
may be as low as 0.5% and as high as about  
20%, the iridium content ranging from about  
2.5% to about 37%, and the rhodium content,  
likewise, ranging from about 2.5% to about 37%.  
I prefer alloys wherein the ruthenium content  
lies between about 1% and a maximum content  
of about 10%. Particularly advantageous are  
alloys within the limits of 80% to 94.5% pal-  
ladium, 1% to 10% ruthenium, 2.5% to 10%  
iridium, and 2.5% to 10% rhodium, such as alloys  
of 80% palladium 5% ruthenium 5% iridium  
and 10% rhodium, or of 90% palladium 2.5%  
ruthenium 2.5% iridium and 5% rhodium.

In order to illustrate the properties of the al-  
loys according to this invention, I may state that  
an alloy of 80% palladium 5% ruthenium 10%  
rhodium and 5% iridium has a tensile strength  
of 133,900 lbs. per square inch when hard, and  
of 94,200 lbs. per square inch when annealed,  
and an elongation of 27% on 2-inches when an-  
nealed. The alloy, likewise, possesses an elec-  
trical resistivity of 200 ohms/mil. ft. The alloys  
in accordance with this invention have higher  
melting point, greater hardness, higher tensile  
strength and higher electrical resistance than  
the alloys described and claimed in my afore-  
said application Serial No. 423,793.

In its best embodiments the alloys consist en-  
tirely of palladium, ruthenium, iridium, and  
rhodium in the proportions specified herein, al-  
though, of course, minor quantities of other met-  
als may be present so long as they do not sub-  
stantially affect the beneficial properties and  
characteristics of my alloys.

What I claim is:

1. An alloy of palladium, ruthenium, iridium,  
and rhodium, comprising 60% to 94.5% palladi-  
um, 0.5% to 20% ruthenium, 2.5% to 37%  
iridium, and 2.5% to 37% rhodium.

2. An alloy of palladium, ruthenium, iridium,  
and rhodium, comprising 80% to 94.5% palladi-  
um, 1% to 10% ruthenium, 2.5% to 10% iridi-  
um, and 2.5% to 10% rhodium.

3. An alloy of palladium, ruthenium, iridium,  
and rhodium, comprising about 80% palladium,  
about 5% ruthenium, about 5% iridium, and  
about 10% rhodium.

CECIL SPENCER SIVIL.